

May 12, 1970

J. W. WARING

3,511,783

SUPERFATTED SOAP BAR CONTAINING A SYNERGISTIC  
PRESERVATIVE MIXTURE OF EHDP AND EDTA

Filed March 7, 1967

3 Sheets-Sheet 1

Fig. 1.



Inventor

John Walter Waring  
By *James J. Kline Jr.*  
Attorney

May 12, 1970

J. W. WARING

3,511,783

SUPERFATTED SOAP BAR CONTAINING A SYNERGISTIC  
PRESERVATIVE MIXTURE OF EHDP AND EDTA

Filed March 7, 1967

3 Sheets-Sheet 2

Fig. 2.



Inventor

John Walter Waring

By *John W. Waring*  
Attorney *John J. Kline, Jr.*

May 12, 1970

J. W. WARING

3,511,783

SUPERFATTED SOAP BAR CONTAINING A SYNERGISTIC  
PRESERVATIVE MIXTURE OF EHDPE AND EDTA

Filed March 7, 1967

3 Sheets-Sheet 3

Fig. 3.



Inventor

John Walter Waring  
By *Donald R. Clark, Jr.*  
Attorney

## 1

3,511,783

SUPERFATTED SOAP BAR CONTAINING A  
SYNERGISTIC PRESERVATIVE MIXTURE  
OF EHDP AND EDTAJohn Walter Waring, Wirral, England, assignor to  
Lever Brothers Company, New York, N.Y., a cor-  
poration of Maine

Filed Mar. 7, 1967, Ser. No. 621,248

Int. Cl. C11d 9/48, 9/34, 9/30

U.S. CL. 252—117

1 Claim

## ABSTRACT OF THE DISCLOSURE

A detergent bar is preserved against deterioration of odour and colour by incorporation of a synergistic mixture of EHDP and EDTA.

This invention relates to detergent bars.

Common faults in a finished bar are that the bar develops spotting or overall discolouration and that the base odour of the detergent deteriorates.

It is generally accepted that the most probable cause of rancidity, deterioration of base odour, in detergent bars, is oxidation of long-chain unsaturated and saturated compounds. The development of spotting or overall discolouration is less clearly understood. It often accompanies deterioration of base odour.

The presence of heavy metals or their salts is known to be an important cause of deterioration of base odour, spotting and discolouration of detergent bars. This cause could be eliminated by ensuring that the ingredients of the bar are free from such metals and that the detergent during its manufacture and processing does not come into contact with them. Since as little as 0.2 part per million copper, in the absence of preservatives, has been shown to have a significant effect on colour and odour deterioration, this solution would be very expensive and so is not satisfactory commercially.

An alternative solution is to use a sequestering agent. The mechanism for the oxidation of long-chain fatty compounds is generally believed to be by a free radical chain reaction. The free radicals required to propagate a chain reaction may be initiated either by traces of heavy metals, or photochemically or thermally. In normal detergent bars, without preservatives, trace metal contamination is responsible for a far higher rate of development of colour and odour than normal amounts of heat and light. Sequestering agents operate by lowering the concentration of heavy metal ions in the bar, and hence lower the rate of free radical initiation.

Other antioxidants frequently used act by absorbing free radicals and thus terminate chain reactions independently of the method of initiation. In this process, the antioxidant is itself destroyed. Thus it is desirable to include a sequestering agent to lower the rate of initiation of free radicals. In addition to the sequestering agent another antioxidant is often included to absorb free radicals initiated by any residual metal ions, or by photochemical or thermal energy sources.

A particular problem is the prevention of deterioration of base odour, spotting and discolouration in super-fatted detergent bars, for example, in soap bars containing significant amounts of free fatty acid.

A typical super-fatted soap contains 10% (calculated as a percentage of the total fatty matter) of free fatty acids but soaps containing 20% of free fatty acid are known. The presence of metal ions, particularly iron and copper ions, in these soaps can be particularly troublesome. Petrolatum, mineral oils, lanoline or other such super-fattening agents can be used as well as fatty acids added separately or specially released in the bar.

## 2

A super-fatted non-soap detergent bar can contain as super-fattening agent a wide variety of compounds. For example, up to 30% of stearic acid has been suggested and other non-fatty acid agents that have been suggested include fatty acid mono-glycerides, long-chain esters of glycols, fatty acid amides, long-chain alkanolamides, in particular isopropanolamides, and long-chain acid sugar esters.

It has now been discovered that by incorporating a mixture of sequestering agents, ethane-1-hydroxy-1, 1-diphosphonic acid, hereafter called EHDP, 1,2-diamino-ethane-N,N·N',N'-tetraacetic acid, commonly called ethylene-diaminetetraacetic acid and hereafter called EDTA, in a detergent bar, a bar is obtained which is especially resistant to the development of rancidity, spotting or overall discolouration.

It is understood that the EHDP, the EDTA or both may be in the form of their esters or, preferably, in the form of their salts. Particularly preferred salts are the alkali-metal, ammonium or triethanolammonium salts.

It has been discovered that a detergent bar that is particularly resistant to the development of rancidity, spotting or overall discolouration can be obtained using a smaller quantity of a mixture of EHDP and EDTA than would be expected from a knowledge of the effect of these compounds separately.

The invention provides a detergent bar containing a synergistic mixture of EHDP and EDTA.

The actual quantity of EHDP and EDTA used will depend to some extent on the particular detergent used but bars according to the invention can be provided by incorporating as little as 0.005% of EHDP in admixture with as little as 0.005% of EDTA. The quantity of EHDP will, in general, be from 0.005% to 0.3% or even higher and that of EDTA 0.005% to 0.3% or higher.

A preferred detergent bar according to the invention contains between 0.01% and 0.08% EHDP and 0.01% and 0.08% EDTA by weight.

A particularly preferred detergent bar according to the invention contains about 0.02% EHDP and about 0.02% EDTA by weight.

The invention is particularly applicable to toilet bars for personal washing.

The invention is even more particularly applicable to super-fatted toilet bars for personal washing. In such bars deterioration in odour and colour is least welcome and the effect of metal ions is most acute as explained above.

Although the invention is particularly applicable to a detergent bar in which the detergent is soap, it will be appreciated that the invention is applicable to any detergent bar that contains an ingredient that contains a long-chain fatty residue. Such ingredients are liable to cause the odour and colour of the bar to deteriorate when metal ions, particularly copper and iron, are also present.

By an ingredient that contains a long-chain fatty residue is meant a compound containing a  $C_{10}$  to  $C_{26}$ , preferably  $C_{12}$  to  $C_{20}$ , group. The chain may be branched but should preferably be straight. The compound will normally contain functional groups, as illustrated below. The  $C_{20}$  to  $C_{26}$  group may contain one or more double bonds.

The invention is, for example, applicable to detergent bars containing, as major active, such non-soap detergents as olefin sulphonates (prepared by the sulphonation of olefins followed by hydrolysis and neutralisation), fatty acyl isothionates, fatty acyl taurides and fatty alcohol sulphates.

It will be appreciated that the invention is also applicable to bars containing mixtures of soap and non-soap detergents. In particular the invention is applicable to bars containing a major proportion of a non-soap detergent together with a minor proportion of soap.

ingredients such as perfumes and other additives can be incorporated into the detergent bars provided by the invention.

When an additive is used, such as a fatty acid alkanolide, that contains a long-chain fatty residue, the mode of action of the invention may be to prevent deterioration in odour and colour of the bar due to the properties of the additive.

The invention will now be illustrated by way of examples.

It should be noted that there is good correlation between the results of long-term tests and the accelerated age tests as used in the examples.

#### EXAMPLE I

Examples of non-superfatted toilet bars according to the invention were prepared and compared with bars containing EHDP and EDTA separately and with bars containing neither EHDP nor EDTA as follows:

##### Method of manufacture: Non-superfatted bars

A large batch of dried soap chips, manufactured from 30% Tallow/20% Palm Kernel Oil fat charge, was thoroughly mixed to ensure homogeneity. Special precautions were taken to minimise metallic contamination in the chips. The batch was sub-divided into 16 sub-batches. To each of 15 of these was added fixed quantities of a solution of EDTA and/or a solution of EHDP. In this 16 batches were obtained with all possible combinations of any one of 4 levels of EDTA (0, 0.03, 0.12 or 0.48%) with any one of 4 levels of EHDP (0, 0.03, 0.12 or 0.48%).

Each of the sub-batches was thoroughly mixed and passed through a three-roll soap mill three times to ensure even distribution of the metal deactivators EDTA and EHDP.

Each sub-batch was then again divided into 3 equal parts. To one part was added 1 p.p.m. copper, in the form of a dilute solution of copper sulphate, and 10 p.p.m. iron in the form of a dilute solution of ferrous ammonium sulphate. Similarly, to the second part 2 p.p.m. copper and 10 p.p.m. iron were added; no additions were made to the third portion. Each of the 48 sub-batches thus produced was thoroughly mixed, milled three times in conventional three-roll soap mills, and extruded through a conventional vacuum refiner plodder.

The final moisture content of the bars was similar to that of conventional toilet soap at 11-12% (total fatty matter 78-79%). Apart from the materials specified, no other ingredients were included; thus the tablets contained no other preservatives or ingredients which are usually included in toilet soaps, such as perfume, preservative, opacifier etc.

The ratio of copper/iron chosen approximates to the average ratio found in practice. Up to 1 p.p.m. copper and 10 p.p.m. iron are frequently found in practice.

##### Methods of storage

Before evaluation of odour each of the toilet bars was stored under one of three different sets of conditions as follows:

(1) 28 days exposed unwrapped in a window to northern sunlight;

(2) 28 days exposed to the atmosphere, unwrapped, at 5°C. in the absence of any illumination; and similarly to (2) at 37°C./25% relative humidity.

##### Method of assessment

Odour was assessed by panels of assistants, experienced in assessing odour in this way, but not especially trained.

The assessment was planned on a statistical basis to ensure the significance of the data to be determined. The 48 bars stored under one set of conditions were compared with one another and the procedure repeated for the other sets of conditions. A design was used in which each bar was compared in turn with each of the other 47

bars. Thus 1128 pairs were compared, each pair twice (once for each order of testing), and each single soap was assessed 94 times. The panel consisted of 113 girls: to avoid fatigue of the olfactory organs, each assistant compared only one pair at a time and not more than 4 pairs during the course of an 8 hour working day. In the comparisons, the panel members were asked to smell the bars with closed eyes (thus to prevent any influence of colour differences) and to express an opinion on "which bar has the stronger odour." Since the samples were unperfumed, this is a direct measure of the strength of the undesirable base odour.

Each answer was scored +1 for the tablet with the strongest odour, 0 for no difference and -1 for that with the weakest odour. The scores for each panel member for each bar were added together to arrive at the total score for each bar. A low score indicates little base odour (good preservation) and a high score indicates strong base odour (poor preservation).

The scores for each of the three sets of storage conditions were added together to give the results given in Table I.

TABLE I

Before addition of further copper and iron:  
Base level of copper, 0.3 p.p.m.  
Base level of iron, 4.6 p.p.m.

| Percent EDTA (No copper/iron added):                 |  | -45  | -111 | -55  | -15  |
|------------------------------------------------------|--|------|------|------|------|
| 0.48                                                 |  | -52  | -85  | -70  | -34  |
| 0.12                                                 |  | -42  | -80  | -67  | 0    |
| 0.03                                                 |  | -7   | -45  | -57  | -53  |
| 0                                                    |  |      |      |      |      |
| Percent EHDP:                                        |  | 0    | 0.03 | 0.12 | 0.48 |
| Percent EDTA (1 p.p.m. copper/10 p.p.m. iron added): |  |      |      |      |      |
| 0.48                                                 |  | +46  | -45  | -43  | -15  |
| 0.12                                                 |  | +141 | -38  | -6   | +24  |
| 0.03                                                 |  | +97  | -123 | -66  | -42  |
| 0                                                    |  | +96  | +04  | +2   | +15  |
| Percent EHDP:                                        |  | 0    | 0.03 | 0.12 | 0.48 |
| Percent EDTA (2 p.p.m. copper/20 p.p.m. iron added): |  |      |      |      |      |
| 0.48                                                 |  | +58  | +4   | -12  | +3   |
| 0.12                                                 |  | +167 | +4   | -37  | +12  |
| 0.03                                                 |  | +107 | +28  | +9   | +6   |
| 0                                                    |  | +120 | +44  | +55  | +128 |
| Percent EHDP:                                        |  | 0    | 0.03 | 0.12 | 0.48 |

Standard error of difference 24.1.  
There is a 19/1 probability of a difference of 48.2 being a true difference.

#### EXAMPLE II

In the following series of bars, covering the use of different levels of copper and iron contamination, a different design pattern was used from that in Example I and the method of manufacture and testing were slightly changed.

##### Method of manufacture: Non-superfatted bars

A large batch of dried soap chips, manufactured from an 80% tallow/20% palm kernel oil fat charge was thoroughly mixed to ensure homogeneity. Special precautions were taken to minimise metallic contamination in the chips. The batch was sub-divided into 30 sub-batches; preservatives and metal contamination were added to each sub-batch at levels defined in the patterns of the attached tables. In each case preservatives were added first and milled into the soap by passing three times through a three-roll soap mill. The metal contaminants, in the form of dilute copper sulphate and ferrous ammonium sulphate solutions, were then added and the soap re-milled in the same way before extrusion through a conventional vacuum refiner plodder. The final moisture content of the bars was similar to that of conventional toilet soap at 11-12%.

## Methods of storage

As described in Example I

## Method of assessment

**Odour.**—The method is essentially as described in Example 1, but the numbers of tests were different to allow for the smaller number of batches.

In each test a design was used in which each of the 30 batches was compared in turn with each of the other 29 batches. Thus 435 pairs were compared, each pair twice (once for each order of testing) and each single soap was assessed 58 times. The panel consisted of 40–45 girls.

Restrictions to avoid olfactory fatigue, questions asked and scoring methods were the same as described in Example 1. In the following tables for individual storage conditions a difference between the scores of 22 is significant at the 95% probability level: i.e. there is a 19/1 probability of a difference of 22 being a true difference. Significance data for tables representing the sum of scores from all storage conditions are given with the tables.

TABLE II

Effect of EHDP and EDTA on Non-superfatted Toilet Bars containing Copper and Iron Contaminants—Total Scores from Panel Test for Odour

Storage conditions: 28 days exposed unwrapped in a window to northern daylight.

Before addition of further copper and iron:

Base level of copper, 0.3 p.p.m.

Base level of iron, 6.5 p.p.m.

| No copper/iron added                  |     |      |     |     |  |
|---------------------------------------|-----|------|-----|-----|--|
| Percent EDTA (as free acid):          |     |      |     |     |  |
| 0.5                                   | +8  |      |     |     |  |
| 0.1                                   | -7  | -14  |     |     |  |
| 0.02                                  | -21 | -20  | -10 |     |  |
| 0                                     | +18 | -4   | -6  | -13 |  |
| Percent EHDP                          |     |      |     |     |  |
| 0                                     | 0   | 0.02 | 0.1 | 0.5 |  |
| 0.5 p.p.m. Copper/5 p.p.m. Iron added |     |      |     |     |  |
| Percent EDTA (as free acid):          |     |      |     |     |  |
| 0.05                                  | +14 |      |     |     |  |
| 0.1                                   | +27 | -8   |     |     |  |
| 0.02                                  | -18 | +2   | -2  |     |  |
| 0                                     | +14 | -6   | -18 | +4  |  |
| Percent EHDP                          |     |      |     |     |  |
| 0                                     | 0   | 0.02 | 0.1 | 0.5 |  |
| 1 p.p.m. Copper/10 p.p.m. Iron added  |     |      |     |     |  |
| Percent EDTA (as free acid):          |     |      |     |     |  |
| 0.5                                   | +26 |      |     |     |  |
| 0.1                                   | +23 | -10  |     |     |  |
| 0.02                                  | +10 | -16  | -1  |     |  |
| 0                                     | +15 | +6   | +1  | +7  |  |
| Percent EHDP                          |     |      |     |     |  |
| 0                                     | 0   | 0.02 | 0.1 | 0.5 |  |

TABLE III

Effect of EHDP and EDTA on Non-superfatted Toilet Bars containing Copper and Iron Contaminants—Total Scores from Panel Test for Odour

Storage conditions: 28 days exposed to the atmosphere, unwrapped, at 45°C. in the absence of any illumination.

Before the addition of further copper and iron:

Base level of copper, 0.3 p.p.m.

Base level of iron, 6.5 p.p.m.

| No copper/iron added                  |     |      |     |     |  |
|---------------------------------------|-----|------|-----|-----|--|
| Percent EDTA (as free acid):          |     |      |     |     |  |
| 0.5                                   | -18 |      |     |     |  |
| 0.1                                   | -1  | +1   |     |     |  |
| 0.02                                  | -3  | -17  | -7  |     |  |
| 0                                     | +21 | +5   | -9  | -14 |  |
| Percent EHDP                          |     |      |     |     |  |
| 0                                     | 0   | 0.02 | 0.1 | 0.5 |  |
| 0.5 p.p.m. Copper/5 p.p.m. Iron added |     |      |     |     |  |
| Percent EDTA (as free acid):          |     |      |     |     |  |
| 0.5                                   | 0   |      |     |     |  |
| 0.1                                   | -3  | +3   |     |     |  |
| 0.02                                  | 0   | -20  | -12 |     |  |
| 0                                     | +14 | +7   | 0   | -14 |  |
| Percent EHDP                          |     |      |     |     |  |
| 0                                     | 0   | 0.02 | 0.1 | 0.5 |  |
| 1 p.p.m. Copper/10 p.p.m. Iron added  |     |      |     |     |  |
| Percent EDTA (as free acid):          |     |      |     |     |  |
| 0.5                                   | 0   |      |     |     |  |
| 0.1                                   | +9  | +7   |     |     |  |
| 0.02                                  | +19 | -8   | -9  |     |  |
| 0                                     | +28 | +30  | 0   | -14 |  |
| Percent EHDP                          |     |      |     |     |  |
| 0                                     | 0   | 0.02 | 0.1 | 0.5 |  |

TABLE IV

Effect of EHDP and EDTA on Non-superfatted Toilet Bars containing Copper and Iron Contaminants—Total Scores from Panel Test for Odour

Storage conditions:

28 days exposed to the atmosphere, unwrapped, at 37°C. 25% relative humidity, in the absence of any illumination.

Before addition of further copper and iron:

Base level of copper, 0.3 p.p.m.

Base level of iron, 6.5 p.p.m.

| No Copper/Iron Added                                                                                                                                                                                                                                                                                                                                         |     |      |     |     |  |
|--------------------------------------------------------------------------------------------------------------------------------------------------------------------------------------------------------------------------------------------------------------------------------------------------------------------------------------------------------------|-----|------|-----|-----|--|
| Percent EDTA (as free acid):                                                                                                                                                                                                                                                                                                                                 |     |      |     |     |  |
| 0.5                                                                                                                                                                                                                                                                                                                                                          | -4  |      |     |     |  |
| 0.1                                                                                                                                                                                                                                                                                                                                                          | 0   | -18  |     |     |  |
| 0.02                                                                                                                                                                                                                                                                                                                                                         | -13 | -1   | -9  |     |  |
| 0                                                                                                                                                                                                                                                                                                                                                            | +32 | +2   | +3  | -5  |  |
| Percent EHDP                                                                                                                                                                                                                                                                                                                                                 |     |      |     |     |  |
| 0                                                                                                                                                                                                                                                                                                                                                            | 0   | 0.02 | 0.1 | 0.5 |  |
| 0.5 p.p.m. Copper/5 p.p.m. Iron Added                                                                                                                                                                                                                                                                                                                        |     |      |     |     |  |
| Percent EDTA (as free acid):                                                                                                                                                                                                                                                                                                                                 |     |      |     |     |  |
| 0.5                                                                                                                                                                                                                                                                                                                                                          | 0   |      |     |     |  |
| 0.1                                                                                                                                                                                                                                                                                                                                                          | 0   | -6   |     |     |  |
| 0.02                                                                                                                                                                                                                                                                                                                                                         | +3  | -5   | -17 |     |  |
| 0                                                                                                                                                                                                                                                                                                                                                            | +25 | +9   | -16 | -12 |  |
| Percent EHDP                                                                                                                                                                                                                                                                                                                                                 |     |      |     |     |  |
| 0                                                                                                                                                                                                                                                                                                                                                            | 0   | 0.02 | 0.1 | 0.5 |  |
| 1 p.p.m. Copper/10 p.p.m. Iron Added                                                                                                                                                                                                                                                                                                                         |     |      |     |     |  |
| Percent EDTA (as free acid):                                                                                                                                                                                                                                                                                                                                 |     |      |     |     |  |
| 0.5                                                                                                                                                                                                                                                                                                                                                          | -7  |      |     |     |  |
| 0.1                                                                                                                                                                                                                                                                                                                                                          | +14 | -7   |     |     |  |
| 0.02                                                                                                                                                                                                                                                                                                                                                         | +1  | -10  | -6  |     |  |
| 0                                                                                                                                                                                                                                                                                                                                                            | +31 | +25  | -5  | -4  |  |
| Percent EHDP                                                                                                                                                                                                                                                                                                                                                 |     |      |     |     |  |
| 0                                                                                                                                                                                                                                                                                                                                                            | 0   | 0.02 | 0.1 | 0.5 |  |
| No Copper/Iron Added                                                                                                                                                                                                                                                                                                                                         |     |      |     |     |  |
| Percent EDTA (as free acid):                                                                                                                                                                                                                                                                                                                                 |     |      |     |     |  |
| 0.5                                                                                                                                                                                                                                                                                                                                                          | -9  |      |     |     |  |
| 0.1                                                                                                                                                                                                                                                                                                                                                          | -8  | -31  |     |     |  |
| 0.02                                                                                                                                                                                                                                                                                                                                                         | -37 | -33  | -26 |     |  |
| 0                                                                                                                                                                                                                                                                                                                                                            | +69 | +3   | -12 | -32 |  |
| Percent EHDP                                                                                                                                                                                                                                                                                                                                                 |     |      |     |     |  |
| 0                                                                                                                                                                                                                                                                                                                                                            | 0   | 0.02 | 0.1 | 0.5 |  |
| 0.5 p.p.m. Copper/5 p.p.m. Iron Added                                                                                                                                                                                                                                                                                                                        |     |      |     |     |  |
| Percent EDTA (as free acid):                                                                                                                                                                                                                                                                                                                                 |     |      |     |     |  |
| 0.5                                                                                                                                                                                                                                                                                                                                                          | +14 |      |     |     |  |
| 0.1                                                                                                                                                                                                                                                                                                                                                          | +24 | -11  |     |     |  |
| 0.02                                                                                                                                                                                                                                                                                                                                                         | -15 | -23  | -31 |     |  |
| 0                                                                                                                                                                                                                                                                                                                                                            | +53 | +10  | -34 | -22 |  |
| Percent EHDP                                                                                                                                                                                                                                                                                                                                                 |     |      |     |     |  |
| 0                                                                                                                                                                                                                                                                                                                                                            | 0   | 0.02 | 0.1 | 0.5 |  |
| 1 p.p.m. Copper/10 p.p.m. Iron Added                                                                                                                                                                                                                                                                                                                         |     |      |     |     |  |
| Percent EDTA (as free acid):                                                                                                                                                                                                                                                                                                                                 |     |      |     |     |  |
| 0.5                                                                                                                                                                                                                                                                                                                                                          | +19 |      |     |     |  |
| 0.1                                                                                                                                                                                                                                                                                                                                                          | +46 | -10  |     |     |  |
| 0.02                                                                                                                                                                                                                                                                                                                                                         | +30 | -33  | -16 |     |  |
| 0                                                                                                                                                                                                                                                                                                                                                            | +74 | +61  | -4  | -11 |  |
| Percent EHDP                                                                                                                                                                                                                                                                                                                                                 |     |      |     |     |  |
| 0                                                                                                                                                                                                                                                                                                                                                            | 0   | 0.02 | 0.1 | 0.5 |  |
| Standard error of difference 19, a difference of 38 is significant at the 95% probability level.                                                                                                                                                                                                                                                             |     |      |     |     |  |
| EXAMPLE III                                                                                                                                                                                                                                                                                                                                                  |     |      |     |     |  |
| The effect of EHDP and EDTA in superfatted bars was assessed as follows.                                                                                                                                                                                                                                                                                     |     |      |     |     |  |
| Method of manufacture: Superfatted soap                                                                                                                                                                                                                                                                                                                      |     |      |     |     |  |
| A large batch of soap was manufactured from a 50% tallow/50% palm kernel oil fat charge and superfatted by the addition of 10% fatty acids (calculated as a percentage of total fatty matter), prepared by acidification of the same soap base. Special precautions were taken to minimise metallic contamination in the final dried superfatted soap chips. |     |      |     |     |  |
| Preparation of the 30 sub-batches was undertaken in exactly the same manner as that of the non-superfatted soaps described in Example II.                                                                                                                                                                                                                    |     |      |     |     |  |
| The storage methods were those used in Example II. Odour was assessed as described in Example I.                                                                                                                                                                                                                                                             |     |      |     |     |  |

Colour was assessed as follows:

Twenty-five girls were asked to rank the bars in each range experiment in order of whiteness. Score 1 for the whitest, 2 for the next whitest and so on. The mean result for each bar is given in the tables.

The odour and colour results obtained are set out in Tables VI to XII.

TABLE VI

Effect of EHDP and EDTA on Superfatted Toilet Bars containing Copper and Iron Contaminants—Total Scores from Panel Test for Odour:  
Storage conditions: 28 days exposed unwrapped in a window to northern daylight.  
Before addition of any further copper and iron:  
Base level of copper, 0.5 p.p.m.  
Base level of iron, 8.9 p.p.m.

| No Copper/Iron Added                  |     |      |     |     |
|---------------------------------------|-----|------|-----|-----|
| Percent EDTA (as free acid):          |     |      |     |     |
| 0.5                                   | +10 |      |     |     |
| 0.1                                   | -2  | -2   |     |     |
| 0.02                                  | -17 | -19  | -15 |     |
| 0                                     | +5  | 0    | -17 | -23 |
| Percent EHDP                          | 0   | 0.02 | 0.1 | 0.5 |
| 0.5 p.p.m. Copper/5 p.p.m. Iron Added |     |      |     |     |
| Percent EDTA (as free acid):          |     |      |     |     |
| 0.5                                   | +23 |      |     |     |
| 0.1                                   | +8  | -13  |     |     |
| 0.02                                  | +9  | -10  | -5  |     |
| 0                                     | +17 | 0    | 0   | -13 |
| Percent EHDP                          | 0   | 0.02 | 0.1 | 0.5 |
| 1 p.p.m. Copper/10 p.p.m. Iron Added  |     |      |     |     |
| Percent EDTA (as free acid):          |     |      |     |     |
| 0.5                                   | +15 |      |     |     |
| 0.1                                   | +14 | +10  |     |     |
| 0.02                                  | +16 | -9   | -7  |     |
| 0                                     | +10 | +13  | -12 | +14 |
| Percent EHDP                          | 0   | 0.02 | 0.1 | 0.5 |

TABLE VII

Effect of EHDP and EDTA on Superfatted Toilet Bars containing Copper and Iron contaminants—Total Scores from Panel Test for Colour:  
Storage conditions: 28 days exposed to the atmosphere, unwrapped at 37° C./25% relative humidity in the absence of any illumination.  
Before addition of any further copper and iron:  
Base level of copper, 0.5 p.p.m.  
Base level of iron, 8.9 p.p.m.

| No Copper/Iron Added                  |     |      |     |     |
|---------------------------------------|-----|------|-----|-----|
| Percent EDTA (as free acid):          |     |      |     |     |
| 0.5                                   | +14 |      |     |     |
| 0.1                                   | +27 | -22  |     |     |
| 0.02                                  | -5  | -9   | 0   |     |
| 0                                     | +19 | -8   | -12 | -6  |
| Percent EHDP                          | 0   | 0.02 | 0.1 | 0.5 |
| 0.5 p.p.m. Copper/5 p.p.m. Iron Added |     |      |     |     |
| Percent EDTA (as free acid):          |     |      |     |     |
| 0.5                                   | +15 |      |     |     |
| 0.1                                   | +29 | -20  |     |     |
| 0.02                                  | +21 | -27  | -13 |     |
| 0                                     | +12 | -4   | -19 | -2  |
| Percent EHDP                          | 0   | 0.02 | 0.1 | 0.5 |
| 1 p.p.m. Copper/10 p.p.m. Iron Added  |     |      |     |     |

| No Copper/Iron Added         |     |      |     |     |
|------------------------------|-----|------|-----|-----|
| Percent EDTA (as free acid): |     |      |     |     |
| 0.5                          | +22 |      |     |     |
| 0.1                          | +20 | -16  |     |     |
| 0.02                         | +25 | -9   | -22 |     |
| 0                            | +23 | +1   | -21 | -16 |
| Percent EHDP                 | 0   | 0.02 | 0.1 | 0.5 |

TABLE VIII

Effect of EHDP and EDTA on Superfatted Toilet Bars containing Copper and Iron Contaminants—Total Scores from Panel Test for Odour:  
Storage conditions: 28 days exposed to the atmosphere, unwrapped at 45° C. in the absence of any illumination.

Before addition of any further copper and iron:  
Base level copper, 0.5 p.p.m.  
Base level of iron, 8.9 p.p.m.

| No Copper/Iron Added                  |      |      |      |     |
|---------------------------------------|------|------|------|-----|
| Percent EDTA (as free acid):          |      |      |      |     |
| 0.5                                   | +5   |      |      |     |
| 0.1                                   | 0    | -10  |      |     |
| 0.02                                  | -31  | -24  | -19  |     |
| 0                                     | 0    | +3   | -6   | -23 |
| Percent EHDP                          | 0    | 0.02 | 0.1  | 0.5 |
| 0.5 p.p.m. Copper/5 p.p.m. Iron Added |      |      |      |     |
| Percent EDTA (as free acid):          |      |      |      |     |
| 0.5                                   | +8   |      |      |     |
| 0.1                                   | +17  | -8   |      |     |
| 0.02                                  | +10  | -9   | -12  |     |
| 0                                     | +4   | +14  | -7   | +1  |
| Percent EHDP                          | 0    | 0.02 | 0.1  | 0.5 |
| 1 p.p.m. Copper/10 p.p.m. Iron Added  |      |      |      |     |
| Percent EDTA (as free acid):          |      |      |      |     |
| 0.5                                   | +14  |      |      |     |
| 0.1                                   | +24  | -4   |      |     |
| 0.02                                  | +21  | -9   | +11  |     |
| 0                                     | +19  | +12  | -9   | +10 |
| Percent EHDP                          | 0    | 0.02 | 0.1  | 0.5 |
| No Copper/Iron Added                  |      |      |      |     |
| Percent EDTA (as free acid):          |      |      |      |     |
| 0.5                                   | +29  |      |      |     |
| 0.1                                   | +25  | -34  |      |     |
| 0.02                                  | -53  | -52  | -34  |     |
| 0                                     | +24  | -5   | -35  | -52 |
| Percent EHDP                          | 0    | 0.02 | 0.1  | 0.5 |
| 0.5 p.p.m. Copper/5 p.p.m. Iron Added |      |      |      |     |
| Percent EDTA (as free acid):          |      |      |      |     |
| 0.5                                   | +44  |      |      |     |
| 0.1                                   | +54  | -41  |      |     |
| 0.02                                  | +40  | -46  | -30  |     |
| 0                                     | +33  | +10  | -28  | -14 |
| Percent EHDP                          | 0    | 0.02 | 0.1  | 0.5 |
| 1 p.p.m. Copper/10 p.p.m. Iron Added  |      |      |      |     |
| Percent EDTA (as free acid):          |      |      |      |     |
| 0.5                                   | +51  |      |      |     |
| 0.1                                   | +58  | -10  |      |     |
| 0.02                                  | +62  | -27  | -18  |     |
| 0                                     | +55  | +26  | -42  | +8  |
| Percent EHDP                          | 0    | 0.02 | 0.1  | 0.5 |
| No Copper/Iron Added                  |      |      |      |     |
| Percent EDTA (as free acid):          |      |      |      |     |
| 0.5                                   | 27.3 |      |      |     |
| 0.1                                   | 23.0 | 7.0  |      |     |
| 0.02                                  | 7.4  | 2.3  | 2.4  |     |
| 0                                     | 18.5 | 7.8  | 11.3 | 2.9 |
| Percent EHDP                          | 0    | 0.02 | 0.1  | 0.5 |
| No Copper/Iron Added                  |      |      |      |     |

TABLE X

Effect of EHDP and EDTA on Superfatted Toilet Bars containing Copper and Iron Contamination—Total Scores (ranking method) from Panel Test for Colour

Storage conditions: 28 days exposed unwrapped in a window to northern daylight.  
Before addition of any further copper and iron:  
Base level of copper, 0.5 p.p.m.  
Base level of iron, 8.9 p.p.m.

| No Copper/Iron Added         |      |      |      |     |
|------------------------------|------|------|------|-----|
| Percent EDTA (as free acid): |      |      |      |     |
| 0.5                          | 27.3 |      |      |     |
| 0.1                          | 23.0 | 7.0  |      |     |
| 0.02                         | 7.4  | 2.3  | 2.4  |     |
| 0                            | 18.5 | 7.8  | 11.3 | 2.9 |
| Percent EHDP                 | 0    | 0.02 | 0.1  | 0.5 |

TABLE X—Continued

| 0.5 p.p.m. Copper/5 p.p.m. Iron Added |       |      |      |      |    |
|---------------------------------------|-------|------|------|------|----|
| Percent EDTA (as free acid):          |       |      |      |      |    |
| 0.5                                   | 29.4  |      |      |      |    |
| 0.1                                   | 25.1  | 13.0 |      |      |    |
| 0.02                                  | 20.8  | 6.5  | 2.7  |      |    |
| 0                                     | 24.0  | 11.8 | 17.0 | 14.6 |    |
| Percent EHDP                          | 0     | 0.02 | 0.1  | 0.5  | 5  |
|                                       |       |      |      |      |    |
| 1 p.p.m. Copper/10 p.p.m. Iron Added  |       |      |      |      | 10 |
| Percent EDTA (as free acid):          |       |      |      |      |    |
| 0.5                                   | 29.7  |      |      |      |    |
| 0.1                                   | 26.6  | 20.2 |      |      |    |
| 0.02                                  | +22.1 | 12.5 | 8.6  |      |    |
| 0                                     | 27.1  | 17.4 | 10.7 | 15.4 |    |
| Percent EHDP                          | 0     | 0.02 | 0.1  | 0.5  | 15 |

TABLE XI

Effect of EHDP and EDTA on Superfatted Toilet Bars containing Copper and Iron Contaminants—Total Scores (ranking method) from Panel Test for Colour  
Storage conditions: 28 days exposed to the atmosphere, unwrapped at 45° C. in the absence of any illumination.  
Before the addition of further copper and iron:  
Base level of copper, 0.5 p.p.m.  
Base level of iron, 8.9 p.p.m.

| No Copper/Iron Added                  |      |      |      |      |    |
|---------------------------------------|------|------|------|------|----|
| Percent EDTA (as free acid):          |      |      |      |      |    |
| 0.5                                   | 22.8 |      |      |      |    |
| 0.1                                   | 22.2 | 5.9  |      |      |    |
| 0.02                                  | 4.6  | 1.6  | 2.6  |      |    |
| 0                                     | 18.6 | 8.2  | 5.5  | 2.0  |    |
| Percent EHDP                          | 0    | 0.02 | 0.1  | 0.5  | 30 |
|                                       |      |      |      |      |    |
| 0.5 p.p.m. Copper/5 p.p.m. Iron Added |      |      |      |      |    |
| Percent EDTA (as free acid):          |      |      |      |      |    |
| 0.5                                   | 26.2 |      |      |      |    |
| 0.1                                   | 26.0 | 12.8 |      |      |    |
| 0.02                                  | 21.0 | 7.9  | 7.4  |      |    |
| 0                                     | 28.8 | 16.4 | 15.4 | 10.8 |    |
| Percent EHDP                          | 0    | 0.02 | 0.1  | 0.5  | 35 |
|                                       |      |      |      |      |    |
| 1 p.p.m. Copper/10 p.p.m. Iron Added  |      |      |      |      |    |
| Percent EDTA (as free acid):          |      |      |      |      |    |
| 0.5                                   | 26.8 |      |      |      |    |
| 0.1                                   | 27.6 | 18.3 |      |      |    |
| 0.02                                  | 24.0 | 12.5 | 11.5 |      |    |
| 0                                     | 30.0 | 20.0 | 11.9 | 15.6 |    |
| Percent EHDP                          | 0    | 0.02 | 0.1  | 0.5  | 40 |

45

TABLE XII

Effect of EHDP and EDTA on Superfatted Toilet Bars Containing Copper and Iron Contamination: Total Scores (ranking method) from Panel Test for Colour  
Storage conditions: 28 days exposed to the atmosphere, unwrapped, at 37° C./25% relative humidity, in the absence of any illumination.  
Before addition of further copper and iron:  
Base level of copper, 0.5 p.p.m.  
Base level of iron, 8.9 p.p.m.

| No Copper/Iron Added                  |      |      |      |      |    |
|---------------------------------------|------|------|------|------|----|
| Percent EDTA (as free acid):          |      |      |      |      |    |
| 0.5                                   | 22.2 |      |      |      |    |
| 0.1                                   | 22.9 | 6.9  |      |      |    |
| 0.02                                  | 5.2  | 1.8  | 4.6  |      |    |
| 0                                     | 9.9  | 2.8  | 5.6  | 3.2  |    |
| Percent EHDP                          | 0    | 0.02 | 0.1  | 0.5  | 55 |
|                                       |      |      |      |      |    |
| 0.5 p.p.m. Copper/5 p.p.m. Iron Added |      |      |      |      |    |
| Percent EDTA (as free acid):          |      |      |      |      |    |
| 0.5                                   | 28.2 |      |      |      |    |
| 0.1                                   | 25.7 | 14.3 |      |      |    |
| 0.02                                  | 20.0 | 10.1 | 10.4 |      |    |
| 0                                     | 26.7 | 12.4 | 10.7 | 12.1 |    |
| Percent EHDP                          | 0    | 0.02 | 0.1  | 0.5  | 65 |
|                                       |      |      |      |      |    |
| 1 p.p.m. Copper/10 p.p.m. Iron Added  |      |      |      |      |    |
| Percent EDTA (as free acid):          |      |      |      |      |    |
| 0.5                                   | 29.0 |      |      |      |    |
| 0.1                                   | 27.0 | 19.0 |      |      |    |
| 0.02                                  | 23.8 | 15.9 | 15.0 |      |    |
| 0                                     | 28.1 | 21.1 | 14.0 | 16.3 |    |
| Percent EHDP                          | 0    | 0.02 | 0.1  | 0.5  | 70 |

75

Table XIII gives the significance data on odour scores.

TABLE XIII

|                              | Standard error of difference | Difference between scores for significance at the 95% probability level |
|------------------------------|------------------------------|-------------------------------------------------------------------------|
| 28 days exposure to daylight | 11.0                         | 22                                                                      |
| 28 days at 45° C.            | 11.0                         | 22                                                                      |
| 28 days at 37° C., 25% R.H.  | 11.0                         | 22                                                                      |
| Sum of scores                | 19.0                         | 38                                                                      |

The significance levels at 95% confidence limits for the colour data are given in FIGS. 1, 2 and 3. These were calculated from the ranking results by statistical analysis.

TABLE XIV

[Key to batch reference numbers for use with FIGS. 1, 2 and 3 for colour]

| No Copper/Iron Added                  |      |      |      |      |  |
|---------------------------------------|------|------|------|------|--|
| Percent EDTA (as free acid):          |      |      |      |      |  |
| 0.5                                   | 2558 |      |      |      |  |
| 0.1                                   | 2556 | 2557 |      |      |  |
| 0.01                                  | 2553 | 2554 | 2555 |      |  |
| 0                                     | 2549 | 2550 | 2551 | 2552 |  |
| Percent EHDP                          | 0    | 0.02 | 0.1  | 0.5  |  |
|                                       |      |      |      |      |  |
| 0.5 p.p.m. Copper/5 p.p.m. Iron Added |      |      |      |      |  |
| Percent EDTA (as free acid):          |      |      |      |      |  |
| 0.5                                   | 2568 |      |      |      |  |
| 0.1                                   | 2566 | 2567 |      |      |  |
| 0.02                                  | 2563 | 2564 | 2565 |      |  |
| 0                                     | 2559 | 2560 | 2561 | 2562 |  |
| Percent EHDP                          | 0    | 0.02 | 0.1  | 0.5  |  |
|                                       |      |      |      |      |  |
| 1 p.p.m. Copper/10 p.p.m. Iron Added  |      |      |      |      |  |
| Percent EDTA (as free acid):          |      |      |      |      |  |
| 0.5                                   | 2578 |      |      |      |  |
| 0.1                                   | 2576 | 2577 |      |      |  |
| 0.02                                  | 2573 | 2574 | 2575 |      |  |
| 0                                     | 2569 | 2570 | 2571 | 2572 |  |
| Percent EHDP                          | 0    | 0.02 | 0.1  | 0.5  |  |

FIG. 1 is for 28 days exposure to northern daylight (Table X).

FIG. 2 is for 28 days at 45° C. (Table XI).

FIG. 3 is for 28 days at 37° C. and 25% relative humidity (Table XII).

In FIG. 1:

0-4.5=very light cream  
4.5-19.2=light cream  
19.2-21.35=cream  
21.35-25.5=dark cream  
25.5-30=very dark cream

In FIG. 2:

0-14=cream  
14-20.3=dark cream  
20.3-23.4=light brown  
23.4-27.1=brown  
27.1-30.0=dark brown

In FIG. 3:

0-11.7=cream  
11.7-21.4=dark cream  
21.4-24.4=light brown  
24.4-30.0=brown

What is claimed is:

1. A superfatted soap bar stabilized against deterioration of odor and color caused by copper and iron contaminants by a synergistic preservative mixture of about 0.02% of ethane-1-hydroxy-1, 1-diphosphonic acid and

11

ut 0.02% of ethylenediamine tetraacetic acid, by  
ght of said bar.

## References Cited

## UNITED STATES PATENTS

214,454 10/1965 Blaser et al. 260—502.4 XR  
224,976 12/1965 Farrar et al. 252—117 XR  
226,330 12/1965 Anstett 252—117

12

3,368,978 2/1968 Irani 252—137  
3,380,924 4/1968 Werdelmann et al. 252—117

LEON D. ROSDAL, Primary Examiner

D. L. ALBRECHT, Assistant Examiner

U.S. Cl. X.R.

252—108, 132

UNITED STATES PATENT OFFICE  
CERTIFICATE OF CORRECTION

Patent No. 3,511,783

Dated May 12, 1970

Inventor(s) John Walter Waring

It is certified that error appears in the above-identified patent and that said Letters Patent are hereby corrected as shown below:

Column 1, line 54 change "in" to --In--.

Column 2, line 25 change "affect" to --effect--.

Column 3, line 21 change "manufacture" to --manufactured--.

Column 5, Table II, subtitle "1 p.p.m. Copper/10 p.p.m. for heading "Percent EHDP" change "9.5" to --0.5--.

Column 5, Table III in heading "1 p.p.m. Copper/10 p.p.m. Iron Added" change "Acded" to --Added--.

Column 6, Example III, line 67 change "fattey" to --fatty--.

Column 9, Table X, subtitle "1 p.p.m. Copper/10 p.p.m. Iron Added" delete "+" from the figure "22.1" in column 1.

Column 10, Table XIV, subtitle "No Copper/Iron Added" under heading "Percent EDTA (as free acid)" change "0.01" to --0.02--.

SIGNED AND  
SEALED  
DEC 8 1970

(SEAL)

Attest:

Edward M. Fletcher, Jr.

Attesting Officer

WILLIAM E. SCHUYLER, JR.  
Commissioner of Patents